

April 25, 1967

R. OWEN

3,315,598

COPYING OF GRAPHIC ORIGINALS

Filed July 28, 1960

FIG. 1



FIG. 2



FIG. 3



FIG. 4



FIG. 5



FIG. 6



INVENTOR  
RICHARD OWEN

BY

Carpenter, Abbott, Coulter & Kinney  
ATTORNEYS

# United States Patent Office

3,315,598

Patented Apr. 25, 1967

1

3,315,598

**COPYING OF GRAPHIC ORIGINALS**  
Richard Owen, North St. Paul, Minn., assignor to Minnesota Mining and Manufacturing Company, St. Paul, Minn., a corporation of Delaware  
Filed July 28, 1960, Ser. No. 45,987  
6 Claims. (Cl. 101—149.2)

This invention relates to the thermographic reproduction of hand-written, typed, printed or other graphic originals. An important aspect of the invention involves the preparation of heat-stable, right-reading reproductions employing conventional visibly heat-sensitive opaque thermographic copy-paper. The invention is directed both to novel processes and to novel compositions and sheet materials.

Thermographic processes for the reproduction of differentially radiation-absorptive graphic originals, as described, for example, in Miller U.S. Patent No. 2,740,896, involve the application to a visibly heat-sensitive copy-sheet of a heat-pattern originating from the brief irradiation of the original with intense radiant energy. The heat-sensitive layer is preferably held in close contact with the printed surface, so as to obtain maximum utilization of the heat-pattern and to provide maximum sharpness and definition of the image-forming areas. One form of copy-sheet accordingly consists of a visibly heat-sensitive coating on a thin flexible transparent backing. Irradiation through the copy-sheet, i.e. by front-printing, and with the sensitive coating in contact with the printed surface, then produces a copy which is viewed through the transparent backing as a right-reading reproduction of the original.

Translucent or opaque backings are available which are adequately transmissive of the radiant energy employed and which are easier to handle than are the thin transparent webs just described. Copy-sheets prepared with such backings may similarly be thermographically front-printed, but the resulting copy is visible only from the coated surface and therefore as a mirror image of the original. Where possible, such copy-papers are therefore ordinarily used for back-printing, which however is limited to use with thin heat-conductive originals printed on one side only.

The present invention in one aspect provides for the preparation, by thermographic front-printing techniques, of right-reading reproductions on opaque, sturdy, easily handled backings.

The visibly heat-sensitive copy-sheets employed in thermographic reproduction remain visibly heat-sensitive in background areas. Subsequent application of heat may therefore distort or obliterate the copy. The present invention makes possible the stabilization of the initial reproduction against subsequent heating, and provides for a permanent copy.

The invention also makes possible the reproduction of graphic originals by lithographic printing techniques using a lithographic master prepared by a process involving thermographic duplication. These and other objects and advantages of the invention are attained by means of an image transfer procedure as hereinafter described and particularly in connection with the accompanying drawings;

FIGURE 1 illustrates conventional thermocopying technique;

FIGURES 2 and 3 illustrate a thermocopying technique in accordance with one embodiment of the present invention;

FIGURES 4 and 5 illustrate a thermocopying technique in accordance with a second embodiment of the present invention wherein the transfer sheet may be used as a lithographic master; and

2

FIGURE 6 illustrates a thermocopying technique in accordance with a third embodiment of the present invention.

FIGURE 1 illustrates conventional thermocopying technique, for example as described in the Miller patent above referred to, in which a graphic original 10 is irradiated with intense radiation from a source 11 through a visibly heat-sensitive copy-sheet 12 having a heat-sensitive layer 13 on a visibly transparent, radiation-transmissive backing 14. The radiation is preferentially absorbed in the inked areas 15, providing a localized heating effect which causes a visible change in corresponding areas 16 of the heat-sensitive layer 13 to produce a right-reading reproduction of the graphic original as viewed through the backing 14.

FIGURE 2, in accordance with the principles of the present invention, the thus treated copy-sheet 12 is next pressed against a heat-activatable sheet 17, having a normally non-tacky, heat-activatable adhesive layer 18 on a backing 19. Heat and pressure are conveniently provided by means of rollers 20, 21 or by other means as desired. The adhesive layer 18 is activated and is adhered to the sensitive coating 13. The composite is next cooled to room temperature, and the backing 14 is stripped away from the sensitive layer 13 which remains adherently bonded to the transfer sheet 17, as shown in FIGURE 3. As viewed from the exposed surface, the sensitive layer 13 provides a direct-reading reproduction of the printed original 10.

When the copy-image is itself radiation-absorptive, a source 11 of radiant energy may alternatively be employed in providing a localized heating effect at the image areas. The adhesive layer 18 is thereby locally activated at those areas in contact with the image areas of the sensitive layer 13 in the composite of FIGURE 2. Pressure may simultaneously be applied by any convenient means, for example through a transparent cover plate or film, or by holding the composite under tension over a convex supporting surface. The image areas are thereby selectively adhered to the adhesive layer. Removal of the backing 14 by stripping then removes the unchanged portions 22 of the sensitive layer 13, leaving the image-forming areas 16 adherently retained by the adhesive layer 18 of the receptor sheet 17, as illustrated in FIGURE 4. Such a copy is no longer visibly changed on further heating.

In those forms of heat-sensitive copy-paper in which the heat-images formed are not preferentially radiation-absorptive, the energy source 11 of FIGURE 1 may still be employed, in conjunction with suitable pressure-applying means, in activating the adhesive layer of the sheet 17 of FIGURE 2. For this purpose, the sheet 17 is itself made radiation-absorptive, e.g. by employing a suitably colored backing 19 or by incorporating small amounts of carbon black or the like in the adhesive layer 18. Since irradiation then causes activation of the entire adhesive layer, the resulting separation occurs as illustrated in FIGURE 3.

In some instances the image-carrying transfer sheet of FIGURE 4 may subsequently be employed as a master sheet in the lithographic duplication of the image. As illustrated in FIGURE 5 there is first applied a coating of a fountain solution 23 which is preferentially accepted by the exposed surfaces of the heat activatable adhesive coating 18, followed by application of a coating of an ink composition 24 which is preferentially accepted by the exposed surfaces of the image areas 16. The ink is then transferred to a receptor sheet as in conventional lithographic duplicating. A negative print is produced where the preferential receptivity of the image and background areas is reversed.

*Example 1*

A heat-sensitive copy-sheet is first prepared by applying a thin uniform layer of a fluid mixture of reagents and binder to thin transparent paper (Ecusta condenser tissue) by knife coating at an orifice of 3 mils, and drying at room temperature. The coating mixture contains the following in parts by weight as indicated:

|                                                                                                                  | Parts |
|------------------------------------------------------------------------------------------------------------------|-------|
| Mixture of equal molar parts of silver behenate and behenic acid dispersed in ethyl acetate at 15% concentration | 10    |
| Ten percent solution of polystyrene resin in acetone, containing added 2% of protocatechuic acid                 | 30    |

The white copy-sheet is placed over a graphic original printed in black ink on white paper, and the composite is momentarily exposed to intense radiation from an incandescent filament in the thermographic copying process hereinbefore noted, producing a copy of the original image in brownish black dense letters on a white background. The exposure is accomplished in a thermocopying machine as described in Kuhrmeyer et al. Patent No. 2,891,165.

A heat-activatable receptor sheet is prepared by applying a thin uniform layer of a mixture of 33 parts by weight of polyvinyl butyral resin, 33 parts of waxy hydrogenated castor oil, 22 parts of liquid chlorinated diphenyl, and 11 parts of 2-biphenyl diphenylphosphate, to 45 pound book paper. The coating is applied at a rate of 18 grams per square foot and at an elevated temperature at which the mixture is fluid. The coating is non-tacky at normal room temperatures but softens and becomes sticky at temperatures of the order of 65° C.

The copy is placed with the imaged coated surface in contact with the coated surface of the receptor sheet and the composite is again passed through the thermocopying machine and briefly intensely irradiated, with the copy toward the source of radiation. The exposure is controlled to provide sufficient heating at the image areas to soften and activate the adhesive coating while avoiding any visible change at the background areas. The composite is then cooled and the paper backing of the copy-sheet is stripped away, taking with it the unchanged and still heat-sensitive coating at the background areas. The visibly darkened image areas of the heat-sensitive coating remain adherently bonded to the receptor sheet.

The heat-sensitive background areas of the copy-sheet may now be visibly changed to a brown-black color by heating, e.g. on a heated plate or in an oven, to produce a negative transparency of the graphic original.

*Example 2*

The heat-sensitive coating of Example 1 is applied to map overlay tracing paper in place of the condenser tissue there employed. A thermographic copy of a graphic original is prepared and the copy placed in contact with the adhesive receptor sheet of Example 1. The composite is subjected to heat and pressure by pressing with a flatiron at a temperature just below that required to cause a visible change in the background areas of the heat-sensitive copy-sheet. After cooling, the tracing paper is stripped away. The entire heat-sensitive layer is found to remain adherently bonded to the receptor sheet.

*Example 3*

In this example a normally non-tacky heat-activatable adhesive composition initially included in the composition of the visibly heat-sensitive coating is transferred to an uncoated paper backing simultaneously with the image-forming components.

Twenty parts by weight of mercuric behenate is first dispersed in a mixture of 48 parts commercial heptane and 32 parts acetone by milling on a ball mill. Separately, one-half part of s-diphenyl carbazide is dissolved in a mixture of 45 parts toluene and 45 parts acetone.

A further solution is prepared of 10 parts of ethyl cellulose and 0.6 part thiourea in 90 parts acetone. The three mixtures are mixed together in the weight ratio of 15:0.5:10, together with 2 parts of diphenyl phthalate, and coated on 30-pound map overlay tracing paper at a coating orifice of 8 mils. After drying at room temperature the coating is non-tacky.

A printed original is placed in heat-conductive pressure-contact with the copy-sheet prepared as just described and is briefly intensely irradiated to produce a visible reproduction of the printed image areas in the heat-sensitive coating. The copy is then placed with the imaged surface against a rough surface bond paper and the composite again irradiated. The image portions of the copy are selectively softened and adhered to the bond paper; on stripping the two sheets apart, a distinct copy of the image remains on the paper, although a major proportion of the image material remains on the copy-sheet. Repeating the same procedure with further sheets of the bond paper produces a number of additional copies before the image material is depleted, as many as eight copies having thereby been prepared.

The transfer step is illustrated in FIGURE 6. The previously imaged portions 16' of the heat-sensitive and heat-activatable layer 13' are selectively softened and adhered to the untreated paper 19, and portions thereof remain on the paper when the copy-sheet 12' is stripped away.

Multiple copies have somewhat analogously been prepared by the methods described in Examples 1 and 2 where the polystyrene resin binder there employed was replaced by a somewhat softer resinous material.

The materials transferred at the image areas in Example 3 are organophilic in nature, whereas the bond paper receptor sheet is hydrophilic. Under these conditions it becomes possible to prepare further copies by lithographic reproduction. The background areas are first coated with an aqueous fountain solution, such as a dilute solution of gum arabic in water, which is selectively retained by these hydrophilic surfaces. Oil-based ink is next applied and is selectively retained by the oleophilic surfaces of the image areas. The ink is then transferred under pressure to a paper receptor, either directly or by means of an intermediate blanket roller. Suitable coated or strengthened hydrophilic sheet materials may replace the bond paper where longer runs are desired.

Lithographic reproduction may also be carried out using heat-activatable adhesive receptor sheets as the lithographic plates, particularly by incorporating in the adhesive layer a hydrophilic component such as a water-soluble gum or a hydrophilic inorganic filler such as silica gel, or by the use of an ink-repellent heat-activatable adhesive such as a waxy water-soluble polyethylene glycol. Systems in which the adhesive coating is oleophilic and the transferred heat-image material is hydrophilic are also contemplated, the copy resulting in this case being a negative rather than a positive copy when using oil-based inks.

What is claimed is as follows:

1. The method of preparing a reproduction of a differentially radiation-absorptive graphic original, comprising: subjecting a heat-sensitive copy-sheet to localized heating at areas corresponding to image-forming areas of said original by a thermographic process to provide a visible reproduction of said image-forming areas, said copy-sheet including a visibly heat-sensitive coating on a flexible carrier; placing said copy-sheet with its coated surface in pressure-contact with the heat-activatable surface of a normally non-tacky adhesive receptor sheet and heating at least the portions of said heat-activatable surface corresponding to said image-forming areas to provide adherent bonding between said coating and said surface while avoiding visible change at background areas of said copy-sheet; and removing said carrier by stripping.
2. The method of preparing a reproduction of a dif-

dentially radiation-absorptive graphic original, comprising: subjecting a heat-sensitive copy-sheet to localized heating by a thermographic process at areas corresponding to image-forming areas of said original to provide a visible reproduction of said image-forming areas, said copy-sheet including a radiation-transmissive flexible carrier and a heat-sensitive coating which is permanently visibly changed and rendered strongly radiation-absorptive when heated in said thermographic process; placing said copy-sheet with its coated surface in pressure-contact with the heat-activatable surface of a normally non-tacky adhesive receptor sheet and briefly strongly irradiating the heat-sensitive coating to cause activation and bonding of said adhesive at image areas while avoiding visible change at background areas of said copy-sheet; and removing said flexible carrier by stripping.

3. The method of making a lithographic master printing plate for multiple reproduction of a graphic original, comprising: subjecting a heat-sensitive copy-sheet to localized heating by a thermographic process at areas corresponding to image-forming areas of said original to provide on said copy-sheet a reproduction of said image-forming areas, said copy-sheet including a flexible carrier and a heat-sensitive coating thereon which is visibly changed and rendered strongly radiation-absorptive when heated in said thermographic process; placing said copy-sheet with its coated surface in pressure-contact with the heat-activatable surface of a normally non-tacky adhesive receptor sheet and briefly strongly irradiating the heat-sensitive coating to cause activation and bonding of said adhesive at image areas while avoiding visible change at background areas of said copy-sheet; and removing said flexible carrier, together with background areas of said heat-sensitive coating remaining attached thereto, by stripping, whereby to expose areas of said adhesive coating corresponding to said background areas; one of said adhesive coating and said heat-sensitive coating being hydrophilic, the other being organophilic.

4. The method of preparing a reproduction of a differentially radiation-absorptive graphic original, comprising: subjecting a heat-sensitive copy-sheet to localized heating by a thermographic process at areas corresponding to image-forming areas of said original to provide a visible reproduction of said image-forming areas, said copy-sheet consisting essentially of a flexible carrier and a heat-sensitive coating thereon which is permanently visibly changed to a strongly radiation-absorptive colored state when heated in said thermographic process and which includes a heat-activatable normally non-tacky soft polymeric binder material; placing said copy-sheet with its coated surface in pressure-contact with a receptor sheet; briefly strongly irradiating the image heat-sensitive coating to cause activation and bonding of said binder material at colored image areas to said receptor sheet while avoiding visible change at background areas of said copy-sheet; and separating said receptor sheet, together with adherently bonded portions of said copy-sheet coating retained thereon, by stripping from said copy-sheet.

5. The method of copying comprising: briefly exposing to intense radiant energy a differentially radiation-absorptive graphic original while in heat-conductive contact with a copy-sheet having a visibly heat-sensitive coating on a flexible carrier, to provide a corresponding differential heat pattern sufficient to form on said copy-sheet a visible copy of said original; placing said copy-sheet with the coated surface in contact with a receptor sheet and heating the composite at least at image areas of said copy to an adhesion-inducing temperature; and stripping from said receptor any portion of said copy-sheet not adherently bonded thereto; at least one of said copy-sheet and said receptor sheet having a thermo adhesive normally non-tacky surface coating which is adhesive when heated to said temperature.

10 6. The method of copying comprising: briefly subjecting a differentially radiation-absorptive graphic original to intense radiation from an incandescent filament while the original is in heat-conductive contact with a copy-sheet product having a heat-sensitive coating, to create at the image areas of said original a heat pattern which is conducted to a copy-sheet and effects a permanent change in said coating at areas corresponding to said image areas; placing the copy-sheet with its said coating in pressure-contact with the surface of a receptor sheet, at least one of said coating and said surface comprising a heat-activatable normally nontacky adhesive bonding material; heating the composite at least at image areas of said copy to an adhesion-inducing temperature for said bonding material, to effect adhesion between said coating and said surface at the heated areas; and separating the copy-sheet and receptor sheet to provide on said receptor a copy of said graphic original.

#### References Cited by the Examiner

##### UNITED STATES PATENTS

|           |         |                  |       |             |
|-----------|---------|------------------|-------|-------------|
| 2,503,758 | 4/1950  | Murray           | ----- | 101-426 X   |
| 2,663,654 | 12/1953 | Miller et al.    |       |             |
| 2,721,821 | 10/1955 | Hoover           | ----- | 156-230     |
| 2,740,896 | 4/1956  | Miller           | ----- | 250-65.1    |
| 2,808,777 | 10/1957 | Roshkind         | ----- | 250-65.1 X  |
| 2,910,377 | 10/1959 | Owen             | ----- | 250-65.1 X  |
| 2,939,009 | 5/1960  | Tien             | ----- | 101-426 X   |
| 2,954,311 | 9/1960  | Vander Weel      | ----- | 101-149.4 X |
| 3,060,023 | 10/1962 | Burg et al.      | ----- | 101-149.4 X |
| 3,063,863 | 11/1962 | Holland et al.   | ----- | 250-65.1 X  |
| 3,109,748 | 11/1963 | Newman           | ----- | 250-65.1 X  |
| 3,121,650 | 2/1964  | Meissner         | ----- | 101-426 X   |
| 3,122,997 | 3/1964  | Raczynski et al. | ----- | 250-65.1 X  |
| 3,129,661 | 4/1964  | Newman           | ----- | 250-65.1    |
| 3,147,377 | 9/1964  | Newman           | ----- | 250-65.1    |

##### FOREIGN PATENTS

|         |        |                |
|---------|--------|----------------|
| 722,023 | 1/1955 | Great Britain. |
|---------|--------|----------------|

ROBERT E. PULFREY, Primary Examiner.

DAVID KLEIN, Examiner.

B. A. LEIGHHEY, E. T. WRIGHT, Assistant Examiners.